



ing textile material according to claim 1, wherein the compound of the said formula is 7-diethylamino-4-methylcoumarin.

3. The method of dry-cleaning and optically brightening textile material according to claim 1, wherein the compound of the said formula is 7-monomethylamino-4-methylcoumarin.

4. The method of dry-cleaning and optically brightening textile material according to claim 1, wherein the compound of the said formula is 7-dimethylamino-4-methylcoumarin.

5. The method of dry-cleaning and optically brightening textile material according to claim 1, wherein the

compound of the said formula is 7-monoethylamino-4-methylcoumarin.

6. The method of dry-cleaning and optically brightening textile material according to claim 1, wherein the compound of the said formula is 7-diethylamino-3,4-di-methylcoumarin.

References Cited in the file of this patent

UNITED STATES PATENTS

|    |           |           |               |
|----|-----------|-----------|---------------|
| 10 | 2,180,508 | De Fraine | Nov. 21, 1939 |
|    | 2,247,259 | Snell     | June 24, 1941 |
|    | 2,333,329 | Miglarese | Nov. 2, 1943  |
|    | 2,341,009 | Axelrad   | Feb. 8, 1944  |
|    | 2,610,152 | Ackermann | Sept. 9, 1952 |